# EUROPEAN PATENT APPLICATION

(11) **EP 1 806 762 A2**
(43) Date of publication of application: **11.07.2007**
(21) Application number: 07250010.1
(22) Date of filing: 03.01.2007
(51) Int. Cl.: H01J 1/32, H01J 17/49

(54) **Plasma display panel and method for producing the same**

(30) Priority: 04.01.2006 KR 20060000849; 06.01.2006 KR 20060001884
(71) Applicant: LG Electronics Inc., Youngdungpo-Gu Seoul (KR)
(72) Inventor: Kim, Bo Hyun, 531-1101 Sinan Apt., Suwon-si Gyeonggi-do, 443-811 (KR); Park, Min Soo, Seocho-gu Seoul, 137-070 (KR); Park, Deok Hai, Joong-gu Daegu, 700-441 (KR); Ryu, Byung Gil, Dongdaemun-gu Seoul, 130-792 (KR); Kim, Young Sung, Yongin-si Gyeonggi-do, 449-722 (KR)
(74) Representative: Camp, Ronald

(57) **Abstract**

A plasma display panel with low firing voltage includes an upper panel (100) and a lower panel (110) facing each other through barrier ribs (112) wherein the upper panel (100) includes a first protective film (380a) composed of magnesium oxide and a second protective film (380b) formed on the first protective film (380a) and composed of a secondary electron-emitting material.

## Description

The present invention relates to a plasma display panel. It more particularly relates to protective films of a plasma display panel.

Plasma display panels include an upper panel, a lower panel, and barrier ribs formed between the upper and lower panels to define respective discharge cells. A major discharge gas, such as neon, helium or a gas mixture thereof, and an inert gas containing a small amount of xenon (Xe) fill the discharge cells. When a high-frequency voltage is applied to produce a discharge in the discharge cells, vacuum ultraviolet radiation is generated from the inert gas to cause phosphors present between the barrier ribs to emit visible light, and as a result, images are created. Such plasma display panels have attracted more and more attention as next-generation display devices due to their small thickness and light weight.

FIG. 1 is a perspective view schematically showing the structure of a plasma display panel. As shown in FIG. 1, the plasma display panel includes an upper panel 100 and a lower panel 110 integrally joined in parallel with and at a predetermined distance apart from the upper panel. The upper panel 100 includes an upper glass plate 101 as a display plane through which images are displayed and a plurality of sustain electrode pairs, each of which consists of a scan electrode 102 and a sustain electrode 103, arranged on the upper glass plate 101. The lower panel 110 includes a lower glass plate 111 and a plurality of address electrodes 113 arranged on the lower glass plate 111 so as to cross the plurality of sustain electrode pairs.

Stripe type (or well type, etc.) barrier ribs 112 for forming a plurality of discharge spaces, i.e. discharge cells, are arranged parallel to each other on the lower panel 110. A plurality of address electrodes 113, which are used to perform an address discharge, are arranged in parallel with respect to the barrier ribs to generate vacuum ultraviolet radiation. Red (R), green (G) and blue (B) phosphors 114 are applied to upper sides of the lower panel 110 to emit visible light upon address discharge, and as a result, images are displayed. A lower dielectric layer 115 is formed between the address electrodes 113 and the phosphors 114 to protect the address electrodes 113.

An upper dielectric layer 104 is formed on the sustain electrode pairs 103, and a protective layer 105 is formed on the upper dielectric layer 104. The upper dielectric layer 104, which is included in the upper panel 100, can become worn out due to the bombardment of positive (+) ions produced during discharge of the plasma display panel. Consequentially, short circuiting of the electrodes may be caused by metal elements, such as sodium (Na). Thus, a magnesium oxide (MgO) protective layer 105 is formed as a thin film on the upper dielectric layer 104 by coating to protect the upper dielectric layer 104. Magnesium oxide sufficiently withstands the bombardment of positive (+) ions and has a high secondary electron emission coefficient, thus achieving a low firing voltage. Accordingly, the protective layer is formed to allow the plasma display panel to be operated at a low voltage. This low-voltage operation leads to a reduction in the power consumption of the panel, thus contributing to a reduction in the production costs of the panel as well as an improvement in the discharge efficiency and brightness of the panel.

However, the protective layer of the conventional plasma display panel has the following problems.

Firstly, magnesium oxide that is currently used as a material for protective layers fails to effectively lower the discharge voltage of plasma display panels on account of its material characteristics. Specifically, the reason for this is that magnesium oxide has a low secondary electron emission coefficient with respect to ions escaping from plasma.

Secondly, secondary electrons can be generated by the bombardment of electrons other than by the bombardment of ions released from plasma. In plasma display panels that are currently produced on an industrial scale, only interactions between ions and magnesium oxide are considered to be important without taking into account the generation of secondary electrons due to the bombardment of electrons.

The present invention seeks to provide an improved plasma display panel.

Embodiments of the invention can provide a plasma display panel with improved secondary electron emission characteristics and a method for producing the plasma display panel.

Embodiments of the invention can provide a plasma display panel with low firing voltage, high brightness, improved discharge efficiency and reduced power consumption, which result from improved secondary electron emission characteristics, and a method for producing the plasma display panel.

Embodiments of the invention can provide a plasma display panel that emits an increased number of secondary electrons due to the bombardment of electrons, and a method for producing the plasma display panel.

Additional advantages and features of the invention will be set forth in part in the description which follows and in part will become apparent to those having ordinary skill in the art upon examination of the following or may be learned from practice of the invention.

In accordance with one aspect of the invention, a plasma display panel includes an upper panel and a lower panel facing each other through barrier ribs wherein the upper panel includes a first protective film composed of magnesium oxide and a second protective film formed on the first protective film and composed of a secondary electron-emitting material.

In accordance with another aspect of the invention, there is provided a method for producing a plasma display panel, the method including forming a first protective film composed of magnesium oxide on a dielectric layer of an upper panel and forming a second protective film composed of a secondary electron-emitting material on the first protective film.

Embodiments of the invention will now be described by way of non-limiting example only, with reference to the drawings, in which:

FIG. 1 is a perspective view of a plasma display panel;

FIG. 2 is a graph showing changes in the firing voltages of different plasma display panels, each of which includes a protective layer composed of magnesium oxide and another oxide; and

FIG. 3 is a view of an upper panel of a plasma display panel according to an embodiment of the invention.

The embodiments of the present invention provide a plasma display panel including a protective layer having a bilayer structure. Hereinafter, a layer formed on one surface of an upper dielectric layer is referred to as a 'first protective film', and a layer formed on the first protective film is referred to as a 'second protective film'.

FIG. 2 is a graph showing changes in the firing voltages of different plasma display panels, each of which includes a protective layer composed of magnesium oxide and another oxide. As is apparent from the graph of FIG. 2, the firing voltages of the plasma display panels can be lowered by the addition of various kinds of oxides other than magnesium oxide to the respective protective layers. FIG. 2 also shows changes in the firing voltages of the plasma display panels with increasing amounts of Y₂O₃, SrO, ZrO₂, ZnO, CaO, Al₂O₃ and TiO₂ added as additives. Although there is a difference depending on the kind of the additives, the firing voltages of the plasma display panels decrease to the lowest values when the number of moles of the additive constituting each of the protective layers reaches about 10% of the total number of moles of the additive and magnesium oxide. Based on these results, the present embodiment provides a plasma display panel including an additional protective film composed of a crystalline oxide. The oxide is not limited to the materials shown in FIG. 2, which have been described for illustration only by way of example.

An explanation of a plasma display panel according to an embodiment of the invention will now be provided with reference to FIG. 3.

The plasma display panel includes sustain electrode pairs 390 included in an upper panel and a dielectric layer 375 formed thereon. Each of the sustain electrode pairs 390 includes a transparent electrode 390a and a bus electrode 390b formed on the transparent electrode. A black electrode 390c is interposed between the transparent electrode 390a and the bus electrode 390b. However, this is not essential to the invention in its broadest aspect. A first protective film 380a and a second protective film 380b are sequentially formed on the first protective film 380a. The first protective film 380a is composed of magnesium oxide, and the second protective film 380b is composed of a secondary electron-emitting material.

A crystalline oxide is used as the secondary electron-emitting material, and a description thereof will be given below.

The crystalline oxide is a material that serves to increase the number of secondary electrons emitted to lower the firing voltage of a plasma display panel. In the present non-limiting embodiment, the crystalline oxide may comprise at least one material selected from alkaline earth metal oxides, alkali metal oxides and transition metal oxides. Examples of alkaline earth metal oxides include MgO, BeO, CaO, SrO and BaO, examples of alkali metal oxides include LiO₂, Na₂O, K₂O, Rb₂O and CsO, and examples of transition metal oxides include TiO₂, Y₂O₃, ZrO₂, Ta₂O₅, ZnO, CoO and MnO. In addition to these materials, Al₂O₃, SiO₂, GeO₂, SnO₂, La₂O₃, CeO₂, Eu₂O₃, Gd₂O₃, etc., may be used as the crystalline oxide. That is, the aforementioned materials must be able to be used to increase the number of secondary electrons emitted by the bombardment of ions upon plasma discharge. The skilled person will be aware of materials other than those specified having properties suitable for use in embodiments of the invention.

In this embodiment the first protective film 380a has a thickness of 400 to 1,000 nm, and the crystalline oxide constituting the second protective film 380b has a size of 50 to 1,000 nm. However these ranges are not essential to the invention in its broadest aspect. In the present embodiment the material of the crystalline oxide may have a shape of a cube or a sphere. If the shape of the crystalline oxide is a cube, the size of the crystalline oxide refers to the length of one side of the cube. On the other hand, if the shape of the crystalline oxide is a sphere, the size of the crystalline oxide refers to the diameter of the sphere. The surface area of the second protective film composed of the crystalline oxide is advantageously as large as possible to increase the number of secondary electrons emitted. Accordingly, it is preferred, but not essential, that the first protective film 380a be not completely covered by the second protective film 380b. Specifically, the surface area of the second protective film 380b is preferably less than 80% and more preferably 30 to 80% of that of the first protective film 380a. However, these ranges of areas are not essential to the invention in its broadest aspect. In the present embodiment the second protective film 380b is formed in such a manner that it has a regular or irregular pattern. However this is not essential.

Particles of the crystalline oxide, e.g., particles of an alkaline earth metal, are formed on the first protective film, and as a result, the surface of the second protective film is rugged rather than flat. Accordingly, the surface area of the second protective film where ions collide upon discharge is increased, resulting in an increase in the number of secondary electrons emitted. This increase in the number of secondary electrons emitted leads to an improvement in the discharge efficiency of the plasma display panel and a reduction in the firing voltage of the plasma display panel. Further, when the second protective film is composed of Gd₂O₃, UV light having a wavelength of about 250 nm is emitted from vacuum ultraviolet (VUV) light of a wavelength of about 147 nm, which is generated from a discharge gas, e.g., Xe, during discharge, resulting in an improvement in the brightness of the plasma display panel.

An explanation concerning the second protective film formed on the first protective film to increase the number of secondary electrons emitted by the bombardment of electrons will now be provided.

In the present exemplary embodiment the second protective film 380b is composed of a material having a secondary electron emission coefficient, which results from the bombardment of electrons, higher than that of magnesium oxide. The material constituting the second protective film 380b may for example be single crystalline or polycrystalline. Examples of such single-crystal materials include KBr, KCl, KI, NaBr, NaCl, NaF, NaI and LiF, and examples of such polycrystalline materials include CsCl, KC1, KI, NaBr, NaCl, NaF, NaI, LiF, RbCl, Al₂CO₃, BaO, BeO, BaF₂, CaF₂, BiCs₃, GeCs, Rb₃Sb, and SbCs₃.

The measured value of secondary electron emission coefficient of magnesium oxide varies depending on the measurement conditions. Magnesium oxide is measured to have a secondary electron emission coefficient lower than 1 under routine conditions. The secondary electron emission coefficients of the single-crystal materials are as follows: KBr = 14, KCl = 12, KI = 10, NaBr = 24, NaCl = 14, NaF = 14, NaI = 19, and LiF = 8.5. The secondary electron emission coefficients of the polycrystalline materials are as follows: CsCl = 6.5, KCl = 7.5, KI = 5.6, NaBr = 6.3, NaCl = 6.8, NaF = 5.7, NaI = 5.5, LiF = 5.6, RbCl = 5.8, Al₂CO₃ = 2-9, BaO = 2.3-4.8, BeO = 3.4, BaF₂ = 4.5, CaF₂ = 3.2, BiCs₃ = 6, GeCs = 7, Rb₃Sb = 7.1, and SbCs₃ = 6. The secondary electron emission coefficient of a material is defined as the number of electrons ejected from the material when one electron collides with the material.

In the present embodiment the first protective film 380a has a thickness of 400 to 1,000 nm, and the single-crystal or polycrystalline oxide constituting the second protective film 380b has a size of 50 to 1,000 nm. However these ranges are given by way of example and are not essential to the invention in its broadest aspect. If the shape of the single-crystal or polycrystalline MgO particles is a sphere, the size of the MgO particles refers to the diameter of the sphere. Conversely, if the shape of the single-crystal or polycrystalline MgO particles is a cube, the size of the MgO particles refers to the length of one side of the cube. The surface area of the second protective film composed of the single-crystal or polycrystalline oxide is advantageously as large as possible to increase the number of secondary electrons emitted. Accordingly, it is preferred, but not essential to the invention in its broadest aspect, that the first protective film 380a be not completely covered by the second protective film 380b. Specifically, the surface area of the second protective film 380b is preferably less than 80% and more preferably 30 to 80% of that of the first protective film 380a. However, these ranges are given by way of example and are not essential to the invention in its broadest aspect. That is, the second protective film 380b is formed on the first protective film 380a such that it has an island shape. Since the material constituting the second protective film 380b is not satisfactorily resistant to the bombardment of ions, the second protective film 380b is formed only on portions of the surface of the first protective film 380a. Accordingly, the magnesium oxide constituting the first protective film 380a functions to protect the second protective film 380b, and the second protective film 380b functions to effectively increase the number of secondary electrons emitted by the bombardment of ions and electrons.

An explanation of a method for producing a plasma display panel according to an embodiment of the invention will now be given.

The method according to this embodiment of the invention is different from conventional methods in that a protective layer having a bilayer structure is formed. Specifically, according to a method according to an embodiment of the invention, a plasma display panel is produced by the following procedure. First, sustain electrode pairs are formed on a glass substrate. Thereafter, a dielectric layer is formed on the glass substrate and the sustain electrode pairs. A first protective film and a second protective film are sequentially formed on the dielectric layer. In this embodiment, the first protective film is composed of magnesium oxide, and the second protective film is composed of a secondary electron-emitting material. The kind and size of the secondary electron-emitting material and the shape of the second protective film are as described in the plasma display panel according to the previous embodiment. That is, the secondary electron-emitting material is a crystalline oxide and is present in the form of particles within the second protective film. Also, the second protective film is composed of a material having a secondary electron emission coefficient, which results from the bombardment of electrons, higher than that of magnesium oxide.

The second protective film composed of crystalline oxide particles is, in the present non-limiting embodiment, formed by preparing a liquid paste, applying the liquid paste to the first protective film, and drying and calcining the applied first protective film. In this embodiment, the liquid paste used to form the second protective film is applied to portions of the surface of the first protective film. In the present embodiment this application of the liquid paste is performed by a process selected from spray coating, bar coating, spin coating, blade coating, and inkjet printing. The liquid paste is prepared by milling a crystalline oxide powder, such as BeO powder, and mixing the milled powder with a solvent and a dispersant. As the amount of the powder increases (i.e. the content of the powder in the final liquid paste increases), the area of the second protective film formed on the first protective film increases. The methods of application are given by way of example only. The skilled person will be aware of other techniques for applying paste and suitable materials for use therewith.

The formation of a second protective film composed of a material having a secondary electron emission coefficient, which results from the bombardment of electrons, higher than that of magnesium oxide is, in this embodiment, achieved by the following procedure. First, a first protective film essentially composed of magnesium oxide is formed by a conventional process selected from e-beam deposition, ion plating, sputtering and screen printing. Subsequently, a second protective film is formed on the first protective film such that it has an island shape. The second protective film may for example be formed by liquid-phase deposition, green sheet lamination or spray coating. When it is intended to form the second protective film having an island shape by green sheet lamination, patterning can be performed in subsequent processing. According to liquid-phase deposition, the concentration of a powder in a liquid paste can be controlled. According to spray coating, the material for the second protective film can be sprayed through a mask disposed on the first protective film. The skilled person will be aware of other techniques suitable for use with the invention.

A method for forming the second protective film by liquid-phase deposition includes preparing a liquid paste, applying the liquid paste to the first protective film, and drying and calcining the applied first protective film. First, a crystalline powder, such as a single-crystal KBr or polycrystalline CsCl powder, is milled. The milled powder is mixed with a solvent and a dispersant to prepare a liquid paste. In the present embodiment, the powder is present in an amount of 1 to 30% by weight with respect to the total weight of the liquid paste, and the dispersant is present in an amount of 5 to 60% by weight with respect to the weight of the powder. As the amount of the powder increases (i.e. the content of the powder in the final liquid paste increases), the area of the second protective film formed on the first protective film increases. These ranges are given by way of example and are not essential to the invention in its broadest aspect.

Subsequently, the liquid paste is applied to the first protective film. The application of the liquid paste can be performed by any suitable technique, such as screen printing, dipping, dye coating or spin coating. Thereafter, the applied liquid paste is dried and calcined to complete the formation of the second protective film. The second protective film thus formed emits an increased number of secondary electrons due to the bombardment of electrons, and as a result, the firing voltage and power consumption of a plasma display panel including the second protective film can be reduced.

It will be apparent to those skilled in the art that, as noted above, various modifications and variations can be made in the embodiments of the present invention without departing from the scope of the invention. Thus, it is intended that the present invention covers the modifications and variations of embodiments of this invention, including, but not limited to, those specifically referred to above, provided they come within the scope of the claims.

## Claims

1. A plasma display panel including an upper panel and a lower panel facing each other through barrier ribs wherein the upper panel includes a first protective film composed of magnesium oxide and a second protective film formed on the first protective film and composed of a secondary electron-emitting material.

2. The plasma display panel according to claim 1, wherein the secondary electron-emitting material is a crystalline oxide and is present in the form of particles within the second protective film.

3. The plasma display panel according to claim 2, wherein the crystalline oxide is at least one material selected from alkaline earth metal oxides, alkali metal oxides, and transition metal oxides.

4. The plasma display panel according to claim 3, wherein the alkaline earth metal oxides are MgO, BeO, CaO, SrO, and BaO.

5. The plasma display panel according to claim 3 or 4, wherein the alkali metal oxides are LiO₂, Na₂O, K₂O, Rb₂O, and CsO.

6. The plasma display panel according to any one of claims 3 to 5, wherein the transition metal oxides are TiO₂, Y₂O₃, ZrO₂, Ta₂O₅, ZnO, CoO, and MnO.

7. The plasma display panel according to any one of claims 2 to 6, wherein the crystalline oxide is at least one oxide selected from Al₂O₃, SiO₂, GeO₂, SnO₂, La₂O₃, CeO₂, Eu₂O₃, and Gd₂O₃.

8. The plasma display panel according to any preceding claim, wherein the second protective film is formed on portions of the surface of the first protective film.

9. The plasma display panel according to any preceding claim, wherein the secondary electron-emitting material has a secondary electron emission coefficient, which results from the bombardment of electrons, higher than that of the magnesium oxide.

10. The plasma display panel according to claim 9, wherein the second protective film is composed of particles of a single-crystal material.

11. The plasma display panel according to claim 10, wherein the single-crystal material is at least one material selected from KBr, KCl, KI, NaBr, NaCl, NaF, NaI, and LiF.

12. The plasma display panel according to any one of claims 9 to 11, wherein the second protective film is composed of particles of a polycrystalline material.

13. The plasma display panel according to claim 12, wherein the polycrystalline material is at least one material selected from CsCl, KCl, KI, NaBr, NaCl, NaF, NaI, LiF, RbCl, Al₂CO₃, BaO, BeO, BaF₂, CaF₂, BiCs₃, GeCs, Rb₃Sb, and SbCs₃.

14. A method for producing a plasma display panel, the method including forming a first protective film composed of magnesium oxide on a dielectric layer of an upper panel and forming a second protective film composed of a secondary electron-emitting material on the first protective film.

15. The method according to claim 14, wherein the secondary electron-emitting material is a crystalline oxide and is present in the form of particles within the second protective film.

16. The method according to claim 15, wherein the second protective film is formed by preparing a liquid paste, applying the liquid paste to the first protective film, and drying and calcining the applied first protective film.

17. The method according to claim 16, wherein the application of the liquid paste is performed by a process selected from spray coating, bar coating, spin coating, blade coating, and inkjet printing.

18. The method according to any one of claims 14 to 17, wherein the secondary electron-emitting material constituting the second protective film has a secondary electron emission coefficient, which results from the bombardment of electrons, higher than that of the magnesium oxide.

19. The method according to claim 18, wherein the second protective film is formed by a process selected from liquid-phase deposition, green sheet lamination, and spray coating.

20. The method according to claim 19, wherein the liquid-phase deposition is performed by preparing a liquid paste, applying the liquid paste to the first protective film, drying the applied first protective film, and calcining the dried first protective film.

21. The method according to claim 20, wherein the area of the second protective film is controlled by varying the concentration of a material in the liquid paste.
